

## UNITED STATES PATENT OFFICE

WILLIS M. PEIRCE AND EDMUND A. ANDERSON, OF PALMERTON, PENNSYLVANIA,  
ASSIGNORS TO THE NEW JERSEY ZINC COMPANY, OF NEW YORK, N. Y., A CORPOR-  
ATION OF NEW JERSEY

## ZINC BASE DIE-CASTING ALLOY

No Drawing.

Application filed August 29, 1930. Serial No. 478,796.

This invention relates to zinc base-die-cast-  
ing alloys and has for its object the provision  
of an improved alloy of this character.

The mechanical requirements of the die-  
casting operation necessitate the construc-  
tion of the melting pot and die from iron and  
steel. These metals are subject to attack by  
molten zinc and it has been found from ex-  
perience that at least 0.25% aluminum must  
10 be added to the zinc in order to minimize this  
attack sufficiently to secure reasonable life  
from the apparatus. Alloys for die-casting  
must possess a sufficient degree of fluidity to  
properly flow into and completely fill the dies  
15 used, and 2% or more aluminum appears to  
be necessary to secure an adequate degree of  
fluidity. It has also long been known that  
aluminum increases the tensile strength of  
20 zinc and this, in itself, makes its presence in  
zinc base die-casting alloys desirable in quan-  
tities of from 2% to as much as 10 to 15%.

Zinc-aluminum alloys containing less than  
about 80% of aluminum undergo a structural  
change subsequent to solidification which is  
25 commonly known as a phase change or more  
specifically in this case as a eutectoid reaction.  
This phase change consists in the formation  
of two crystalline forms or phases from one  
30 phase previously existing, and is accompanied  
by certain changes in physical properties of  
the alloy, such, for example, as increase in  
density, hardness and tensile strength and  
decrease in ductility and impact strength.

35 This phase change may occur during the  
cooling of the alloy after casting or may  
through certain influences be retarded or in-  
hibited. In such cases it may take place  
gradually over a period of months at ordi-  
40 nary temperatures.

A secondary stage of phase change which  
sometimes occurs is the growth of coalescence  
of the extremely small particles of the new  
phases as first formed into larger particles.  
45 This stage may be accompanied by softening

or lowering of tensile strength and by an in-  
crease in ductility and impact strength.

Zinc-aluminum alloys in this range of com-  
position are also subject to a type of disinte-  
gration commonly known as intercrystalline 50  
oxidation. In extreme cases, under the in-  
fluence of warmth and moisture, intercrystal-  
line oxidation may completely penetrate  
specimens of these alloys and cause swelling,  
warping and even complete disintegration. 55  
Intercrystalline oxidation is in some way  
associated with and partly dependent upon  
the phase change.

It has heretofore been recognized that cer-  
tain other metals when present in these zinc-  
aluminum alloys exercise important effects  
on either the phase change or the intercrystal-  
line oxidation or both. For example, copper  
and magnesium are known to exert an in-  
fluence on the phase change either in respect  
60 to the rate at which it takes place or the com-  
pleteness of the reaction or in some other re-  
spect not fully understood. The particular  
effect produced by copper and magnesium on  
the phase change reacts favorably in increas-  
ing the resistance of the alloys to intercrystal-  
line oxidation. Lead, while not exerting any  
marked influence on the phase change, very  
seriously diminishes the resistance of these  
zinc-aluminum alloys to intercrystalline oxi-  
dation. Cadmium, though having a certain  
70 effect on the phase change, in the presence of  
lead usually diminishes the resistance of these  
alloys to intercrystalline oxidation.

Zinc base alloys suitable for die-casting are 75  
known and in use. An alloy containing 4%  
aluminum, 3% copper and the balance high  
grade zinc metal has been widely used and  
is satisfactory for many purposes. This alloy  
is, however, open to two objections. First, 85  
upon ageing, either at normal temperatures  
or at slightly elevated temperatures, the alloy  
suffers a serious loss in impact strength and a  
change in linear dimensions. Secound, in the  
presence of moisture, and particularly in the 90

presence of warmth and moisture together, the alloy undergoes intercristalline oxidation which causes serious changes in physical properties and dimensions.

5 In the course of an exhaustive investigation of zinc base die-casting alloys, we have found that the tendency of zinc-aluminum alloys to undergo intercristalline oxidation is greatly diminished by the elimination of 10 harmful impurities notably lead and tin and under certain conditions cadmium. This was taken advantage of in the preferred composition of the alloy described in the United States patent of Peirce and Anderson No. 15,967,61, dated August 17, 1926 by the use of high grade zinc metal (e. g. Horsehead brand) as the zinc base of the alloy. High grade zinc metal, however, contains as much as 0.05% of lead and to produce an alloy sufficiently free from intercristalline oxidation with this amount of lead present additions of both copper and magnesium are necessary since these metals individually tend to retard or prevent intercristalline oxidation and when present together have a more or less additive beneficial effect.

Continued experiments with zinc metal containing materially less lead than present in high grade zinc metal indicated definitely 30 that there were important possibilities in this direction. We have now discovered that if the percentage of lead and other impurities in the zinc metal (used in making up the zinc base alloy) is less than 0.02% with tin 35 substantially absent, the presence of copper in excess of 2% but not exceeding about 6% (and without magnesium very materially retards intercristalline oxidation, and that such an alloy has a wide field of application as a 40 die-casting metal.

Our present invention accordingly contemplates a zinc base die-casting alloy substantially free of magnesium and containing from about 2 to 10% aluminum, copper in excess of 2% and not exceeding 6%, and in which the zinc base is zinc metal of high purity containing at least 99.98% zinc and preferably containing 99.99+ % zinc. Our present preferred composition of the alloy of the invention is about 4% aluminum, about 3% copper and the balance zinc metal of high purity containing 99.99+ % zinc. The zinc metal of high purity should contain not more than about 0.01% lead plus cadmium. Very satisfactory results have been secured with zinc metal containing 99.99+ % zinc, less than 0.003% lead, less than 0.003% cadmium and less than 0.001% tin. Tin should be substantially excluded from the alloy and in no case should the tin content exceed about 0.001%.

The following table illustrates the important physical properties of a die-casting made of an alloy of the invention. Alloy No. 1 is 65 of the composition heretofore largely used

as a zinc base die-casting alloy made up of high grade zinc metal. Alloy No. 2 is an alloy of the invention:

| Composition               |             |                              | 70 |
|---------------------------|-------------|------------------------------|----|
|                           | Alloy No. 1 | Alloy No. 2                  |    |
| Aluminum.....             | 4.0%        | 4.0%                         |    |
| Copper.....               | 3.0%        | 3.0%                         |    |
| Quality of zinc base..... | High grade  | High purity<br>(99.99+ % Zn) | 75 |

| Properties as cast           |             |             |    |
|------------------------------|-------------|-------------|----|
|                              | Alloy No. 1 | Alloy No. 2 |    |
| Tensile strength, flat.....  | 41,300      | 44,500      |    |
| Tensile strength, round..... | 42,600      | 43,100      |    |
| Impact strength.....         | 132         | 146         | 80 |

| Properties after ten days in steam at 95° C. |             |             |    |
|----------------------------------------------|-------------|-------------|----|
|                                              | Alloy No. 1 | Alloy No. 2 |    |
| Tensile strength, flat.....                  | 9,600       | 32,900      |    |
| Tensile strength, round.....                 | 13,300      | 37,400      |    |
| Impact strength.....                         | 5           | 10          | 85 |
| Expansion $\frac{3}{4}$ " wide.....          | 0.0201      | 0.0047      |    |
| Expansion $\frac{1}{2}$ " wide.....          | 0.0131      | 0.0044      |    |

The tensile strength is indicated in pounds per square inch for flat and round test specimens. The impact strength is indicated in foot pounds per square inch. Linear expansion is indicated in inches for test sections  $\frac{3}{4}$  in. and  $\frac{1}{2}$  in. in width.

We claim:

1. A zinc base alloy consisting of 2 to 10% aluminum, copper in excess of 2% but not exceeding 6%, and the balance zinc metal of high purity containing less than 0.01% of lead plus cadmium.

2. A zinc base alloy consisting of about 4% aluminum, about 3% copper and the balance zinc metal of high purity with at least 99.98% zinc.

3. A zinc base alloy composed of 2 to 5% aluminum, copper in excess of 2% but not in excess of the aluminum, and in which the zinc base is zinc metal of high purity containing at least 99.98% zinc.

In testimony whereof we affix our signatures.

WILLIS M. PEIRCE.  
EDMUND A. ANDERSON.

118

120

125

130